

## UNITED STATES PATENT OFFICE

2,001,474

## PROCESS OF TIN PLATING

Francis H. Snyder, Niagara Falls, N. Y., and  
 Stanley F. M. MacLaren, Niagara Falls, Ontario,  
 Canada, assignors to Industrial Research, Lim-  
 ited, Niagara Falls, Ontario, Canada, a corpo-  
 ration of Ontario

No Drawing. Application November 10, 1931,  
 Serial No. 574,226

3 Claims. (Cl. 91—70.2)

This invention relates to an improved "tin plating" process and more particularly to an improved process of coating light gauge sheet metal, such as thin sheet iron, with a corrosion resisting tin-cadmium alloy.

The principal object of the present invention is to provide an improved process of coating thin gauge sheet metal for use in the manufacture of so-called tin cans.

10 An important object of the invention is to provide thin gauge iron sheets plated with a corrosion resisting tin-containing alloy which are bright and attractive in appearance and which are particularly adapted to be fabricated into containers in which foods may be safely packed without further coating of the metal as with lacquer or the like.

15 Other objects and advantages of the invention will become apparent during the course of the following description.

20 As is well known, it is customary practice in the manufacture of so-called tin cans and tin containers in which articles of food are to be packed to apply to the interior surfaces of the cans or containers a protective coating such as a lacquer in order to prevent the formation of deleterious ingredients in the food as a result of the reaction between compounds present in the food with the metal from which the cans and containers are made. This practice of lacquering the interiors of such containers was necessitated primarily by the fact that the processes customarily used in plating thin gauge sheet metal were not successful in entirely covering the base metal. For example, the ordinary tin containers in general commercial use will often contain so-called "pinholes" as a result of the imperfect covering of the base metal with the tin coating.

25 Although there has been somewhat of an unfavorable reaction by the public to the dark appearing surfaces of lacquered cans and containers manufacturers have been unwilling to discontinue the lacquering process because of the possible dangers to health resulting from packing certain fruits and meat products in unlacquered containers. By the use of the present invention the use of lacquers and similar protective coatings may be safely eliminated thereby saving the expense of the separate lacquering process as well as providing cans and containers having bright, attractive surfaces.

30 In the practice of the present invention the sheets of thin gauge iron to be plated are first given a fast bright pickle according to any of the usual pickling processes now employed for this

purpose. Thereafter the sheets are washed thoroughly with water and are promptly immersed in a suitable solution, such as zinc chloride, to prevent the action of the air or other oxidizing agent thereon.

35 The pickled and washed sheets are plated by dipping them in a molten mass of a tin-cadmium alloy. In preferred practice the alloy consists of 90 per cent. tin and 10 per cent. cadmium by weight. The cadmium content may be varied from about 1 per cent. to approximately 50 per cent. but we have found that there is no practical advantage in employing substantially more than 10 per cent. cadmium and that the results of the plating are somewhat less satisfactory as the cadmium content approaches 1 per cent. In the preferred operation of the process the temperature of the molten mass is maintained around 220° C. although this temperature may be varied considerably. Obviously the temperature must be sufficient to maintain the mass in molten condition during the period of treatment but the use of a temperature substantially in excess of 220° C., while practical in some instances, is disadvantageous in that excessive splashing of the molten metal results. Moreover, too thin a film of alloy is deposited when a temperature substantially in excess of the preferred temperature is employed.

40 In order to reduce the possibility of oxidation during the treatment it is advisable to add to the molten metal a flux which has a melting point below the operating temperature of the process. Various fluxes may be employed but we recommend the use of a flux consisting of 80 per cent. zinc chloride, 15 per cent. sodium chloride and 5 per cent. potassium chloride, the percentages being calculated in parts by weight.

45 The time of treatment of the metal sheets in the molten mass may be varied considerably depending upon the temperature of operation, the alloy used and the thickness of the coating desired. Where, as in the preferred practice, an alloy of 90 per cent. tin and 10 per cent. cadmium is employed with a flux of the type referred to above and the process is operated at a temperature of about 220° C. it is necessary to immerse the sheets in the molten bath for only about two or three minutes. Following the coating of the sheets in the molten bath they are "wiped" to the desired thinness of film according to conventional practice. Thereupon the sheets are quenched with water in conventional manner, after which the sheets are ready for use as desired.

50 As indicated above the treatment described im-

parts a bright surface to the metal and provides a coating which uniformly and completely covers the base sheet metal so that the plated metal may most advantageously be used in the manufacture of tin cans and like containers for packing food products therein. One of the most important advantages of the process is that the plated metal produced is entirely inert with respect to fruit acids and other constituents in food products which are customarily packed in tin containers with the result that it is wholly unnecessary to apply to the inner surfaces of containers made from metal prepared in accordance with the present process an additional coating of lacquer or the like.

While we have described in detail the preferred practice of our invention, it is to be understood that the details of procedure may be variously modified without departing from the spirit of the invention or the scope of the subjoined claims.

We claim:

1. The process of manufacturing plated light gauge metal sheets to be used in the manufacture of cans and the like which comprises cleaning the surface of the metal sheet under treatment, and applying a corrosion resisting coating to the cleaned sheet by immersing the same in a molten

bath of an alloy consisting of approximately 10 per cent. cadmium and 90 per cent. tin.

2. The process of manufacturing plated light gauge iron sheets to be used in the manufacture of cans and the like which comprises subjecting the iron sheets to a fast bright pickle, and subsequently applying a corrosion resisting coating to the sheets by immersing the same for approximately two or three minutes in a molten bath of an alloy consisting of approximately 10 per cent. 10 cadmium and 90 per cent. tin, said bath being maintained at a temperature of approximately 220° C. during the treatment, removing the sheets from the bath, "wiping" the sheets to provide a metal film of the desired degree of thickness, and 15 quenching the thus treated sheets in water.

3. The process of manufacturing plated light gauge metal sheets to be used in the manufacture of cans and the like which comprises cleaning the surface of the metal sheet under treatment, and 20 applying a metal coating to the cleaned sheet by immersing the same in a molten bath of an alloy consisting of cadmium and tin, the cadmium constituting approximately from 1 to 10 per cent. by weight of said alloy.

FRANCIS H. SNYDER.

STANLEY F. M. MACLAREN.